

(No Model.)

W. N. CORNELL.  
PROCESS OF PREPARING WOOD PULP.

No. 433,326.

Patented July 29, 1890.



Witnesses

Horis A. Clark

A. T. Middleton

Inventor

William N. Cornell

by  
Francis L. Dyer  
Attorney

# UNITED STATES PATENT OFFICE.

WILLIAM N. CORNELL, OF PULASKI, NEW YORK.

## PROCESS OF PREPARING WOOD PULP.

SPECIFICATION forming part of Letters Patent No. 433,326, dated July 29, 1890.

Application filed June 26, 1886. Renewed June 28, 1890. Serial No. 357,089. (No specimens.)

*To all whom it may concern:*

Be it known that I, WILLIAM N. CONNELL, a citizen of the United States, residing at Pulaski, in the county of Oswego and State of New York, have invented certain new and useful Improvements in the Process of Preparing Wood Pulp; and I do hereby declare the following to be a full, clear, and exact description of the invention, such as will enable others skilled in the art to which it appertains to make and use the same.

My invention relates to a new and improved process whereby I am enabled to accurately imitate various varieties of wood in wood pulp, and in the carrying out of which I am enabled to make use of an ordinary wood-pulp machine with several additions thereto, so that it is possible to form sheets of wood pulp with a natural grain imprinted thereon as readily and as economically as plain sheets.

For a better understanding of my improved process attention is invited to the accompanying drawings, forming a part of this application, and in which—

Figure 1 is a side elevation of a well-known form of wood-pulp machine, showing my attachment thereto for the carrying out of my improved process; and Fig. 2, a perspective view of the upper press-roll for forming the impression.

The machine shown in Fig. 1 of the drawings, it should be understood, is merely to illustrate the manner of carrying out one step of my improved process, and it should also be understood that any other well-known wood-pulp machine can be used for that purpose. In the machine shown, however, the following parts are represented:

A is the vat or trough within which the disintegrated and saturated pulp is placed.

B is the making-cylinder, working in the pulp and which carries a thin layer of pulp continuously to the felt or apron J. This felt or apron J passes around the roller C and over small auxiliary rollers D D, mounted upon the frame-work, which is supported, in the usual way, upon suitable legs or standards E E.

The rollers C and several of the auxiliary rollers D D are mounted so as to be capable of moving longitudinally in their respective bearings, as is common in many classes of machinery, so that the felt J can be kept always

very taut. The felt or apron J passes between the two rollers G and H, respectively, mounted horizontally upon a suitable standard F and provided with ordinary mechanism for increasing the pressure between the two. The lower roll is of the usual construction, but the upper press-roll (shown in enlarged view of Fig. 2) is made of the wood that is to be imitated, and its outer surface is of the natural condition of the wood in contradistinction from a planed or artificially-smoothed surface. A suitable metal-roll matrix carved or engraved with the grain may be used in place of the wood that is to be imitated.

Power can be applied for moving the felt or apron and making-cylinder B either to the roll C, auxiliary rollers D D to the roller C, or to the making-cylinder.

Partially with the apparatus illustrated, and which has been just described, my improved process is carried out as follows: The pulp is first disintegrated in any usual form of beating-engine and is placed within the vat A, mixed with water in the usual way. To the pulp in this condition is added a sufficient quantity of coloring-matter, so as to color the pulp of the exact tint of the wood that is to be imitated. This coloring-matter can be of any variety desired, either mineral or vegetable pigments, and, if need be, may be applied in the beating-engine instead of in the vat. The felt and making-cylinder being now set in motion, a very thin layer of the watery pulp will adhere to the surface of the making-cylinder and will be carried up and taken off by the felt J. This thin layer of pulp is carried by the felt to the press-rolls and is taken up by the upper press-roll, and is wound convolutionally thereon until a sufficient thickness of pulp is wound on said upper press-roll, when it is cutoff by the usual cutting-knife I. Now, as each thin layer of pulp is wound on the upper press-roll, it is imprinted in relief and depression with the impression of said roll, which is, it will be remembered, the exact wood that is to be imitated, or of metal suitably carved or engraved. The roughened surface of the upper press-roll in pressing against the thin layer of pulp as they are wound thereon causes a peculiar action in the coloring-matter therein, which is as follows:

The relief portions or streaks which are light-

est colors in the press-roll in forcing the pulp to assume their form also squeeze or press the coloring-matter with which they come into contact into those portions of the 5 pulp where there is no pressure—*i. e.*, where the corresponding portions of the press-roll are depressed and are darker colored—so that it will be seen the pulp will be covered exactly like the natural wood. In this way I 10 imprint every layer of pulp that is wound on the upper press-roll with the exact counterfeit of a natural grain and of the exact color of the wood, and as each layer is wound over the one directly beneath the configuration of 15 the press-roll is impressed on and colors the various layers exactly the same, so that the impression of the wood will extend entirely through the pulp. The pulp when removed is first dried in a suitable drying-loft or by other 20 means. It is then preferably calendered by any of the well-known processes, after which it is sandpapered and varnished. In this 25 way I am enabled to obtain a very correct imitation of almost any of the well-known varieties of woods, and by means of the final finishing operations—*viz.*, calendering, sandpapering, and varnishing the resultant article is 30 of a high polish and is a handsome and salable article. It will be evident, however, that such 35 final operations can be dispensed with, if necessary; but I have found by making use of the same that the article is of a much better finish.

In the above description, irrespective of a 35 machine, it will be evident that my process consists, generally, as follows: in, first, beating and coloring the pulp; in, second, carrying the thin layer to the press-rolls; in, third, winding the thin layers convolutionally

40 around a press-roll made of the configuration of the wood to be imitated; in, fourth, drying the pulp; in, fifth, calendering the same; in, sixth, sandpapering the sheet, if desired, and, finally, in varnishing the pulp, all which will be embraced in my claims.

45 Having now described my invention, what I claim as new therein, and desire to secure by Letters Patent, is as follows:

1. The process of preparing wood pulp in imitation of wood, which consists in beating 50 the pulp and then coloring the pulp of the color of the wood that is to be imitated, and afterward forming it into sheets or boards by winding it convolutionally around a press-roll made of the configuration of the wood 55 that is to be imitated, so that the grain and irregularities of the face of the roll will be imprinted upon each convolutional layer on the roll and the pulp will be colored, substantially as set forth.

60 2. The process of preparing wood pulp in imitation of wood, which consists in beating the pulp and then coloring the pulp of the color of the wood that is to be imitated, and afterward forming it into sheets or boards by 65 winding it convolutionally around a press-roll made of the configuration of the wood that is to be imitated, so that the grain and irregularities of the face of the roll will be imprinted upon each convolutional layer on 70 the roll, and then drying, calendering, and sandpapering such sheets or boards.

75 In testimony whereof I affix my signature in presence of two witnesses.

WILLIAM N. CORNELL.

Witnesses:

L. J. CLARK,  
F. D. JOHNSON.